

Feb. 26, 1946.

**D. EDGE**

**2,395,729**

## PRODUCTION OF FERROUS SULPHATE MONOHYDRATE

Filed Feb. 5, 1944



INVENTOR:  
*DEXTER EDGE,*  
BY: *John E Jackson*  
ATTORNEY.

## UNITED STATES PATENT OFFICE

2,395,729

## PRODUCTION OF FERROUS SULPHATE MONOHYDRATE

Dexter Edge, Gary, Ind.

Application February 5, 1944, Serial No. 521,253

4 Claims. (Cl. 23—126)

This invention relates to the production of ferrous sulphate monohydrate, and more particularly to the recovery thereof from waste pickle liquor and is a continuation-in-part of my patent application No. 422,304, filed December 9, 1941.

In the cleaning of various metallic articles, there is used a pickling solution comprised of sulphuric acid. From this pickling solution there results a product known as "pickle liquor" which includes in solution iron and acid.

For a number of years the disposition of pickle liquor has been an acute problem. One method of disposal is to treat it in such manner as to produce ferrous sulphate monohydrate. For the most part, these operations have been on a laboratory scale, but they have successfully demonstrated that the monohydrate can be produced.

The disposal of pickle liquor is more involved than merely removing the ferrous sulphate monohydrate; for example, copper-bearing steels are frequently pickled, and in such case it is necessary to remove the resultant copper sulphate from the pickle liquor.

It is known that the solubility of copper sulphate increases with the temperature, and this characteristic indicates that around 290° F. to 350° F. the ferrous sulphate monohydrate will settle out and leave the copper sulphate in solution.

One method which may be employed for the commercial production of ferrous sulphate monohydrate relies upon the principle of sedimentation, but so far as I am aware it has been confined to treatment in batches. It is apparent that such a method of manufacture is limited in output due to the time required to bring each batch to reaction temperature, settling, removing emptying, and replacing the receptacles. In addition, unusual precautions must be taken to provide equipment which can be safely handled to prevent serious burning of the operators by hot liquid at high pressures, such as a temperature of around 350° F. and pressures in the nature of 120—140 pounds per square inch.

At the cooling end, ferrous sulphate exists as 7(H<sub>2</sub>O)FeSO<sub>4</sub>; at the peak solubility as 4(H<sub>2</sub>O)FeSO<sub>4</sub>, and at the high temperature end as 1(H<sub>2</sub>O)FeSO<sub>4</sub>, the monohydrate being completely insoluble at 290° F.

It has previously been proposed, in the treatment of waste pickle liquor, to use the cooling end to form FeSO<sub>4</sub> crystals, but if the cooling plan is used the copper sulphate and iron sulphate will both settle out as crystals, which will be contaminated. The cooling method also requires ice ma-

chinery. In addition, the combined heat and cooling cycle results in excessive heat loss.

It is among the objects of the present invention to produce ferrous sulphate monohydrate from waste pickle liquor by adopting the high-temperature crystallization of the monohydrate whereby there is permitted, if desired, electrolytic copper refining to remove any copper sulphate from the returning pickle liquor which has been freed of ferrous sulphate.

Another object is to provide a method of the foregoing type which is well adapted to an effective heat cycle such as will allow heat exchanges to maintain temperature levels at each point at the minimum heat required.

Another object is to provide a continuous system of production which will permit the uninterrupted return of the pickle liquor after the ferrous sulphate has been removed.

The invention, then, comprises the features hereinafter fully described and as particularly pointed out in the claims, the following description and the annexed drawing setting forth in detail a certain illustrative embodiment of the invention, this being indicative of one of the number of ways in which the principles of the invention may be employed.

In said drawing, the single figure is a diagrammatic view of the apparatus of the present invention, illustrating the sedimentation tank and its heating instrumentalities in section.

Referring more particularly to the drawing, wherein there is illustrated apparatus which may be employed in the practice of the present invention, the numeral 2 designates a pickling tank through which the workpiece, such as strip metal X, is adapted to be passed and pickled in accordance with well-known practice. This pickling tank 2 is supplied with make-up pickling acid through a pipe 3. Communicating with the bottom of the pickling tank 2 is an outlet pipe 4 which passes through a heat exchanger 5 and connects with a waste pickle liquor manifold 6. Through a pipe 7, the waste pickle liquor manifold 6 is connected to a waste pickle liquor storage vat 8.

A pump 10 is connected to the waste pickle liquor storage vat 8, and serves to boost the waste pickle liquor to a pressure of about 160 pounds per square inch and force it through a pipe 13 which passes through a heat exchanger 14, steam heater 15, and enters the top of a sedimentation tank 16.

Within the sedimentation tank 16 and adjacent the top thereof is a discharge nozzle 17

which is connected to the end of the pipe 13. This discharge nozzle 17 is mounted within a large conical baffle 18 which is in spaced relationship with respect to the walls of the upper portion of the sedimentation tank 16, and the lower portion of the baffle 18 is provided with a flared skirt 19 which extends into close proximity to the walls of the sedimentation tank, and whose sloping outer surface forms one side of a passageway 20 located between the skirt and wall of the tank 16.

The lower portion 21 of the sedimentation tank 16 is of inverted cone shape, and terminates in a discharge opening 22. Mounted in this discharge opening 22 is a float controlled valve 23 which is disposed over the opening or expanding nozzle 25 of a collecting chamber 26. The nozzle 25 is so shaped as to permit rapid separation or escape of steam from the discharged crystals. Associated with this collecting chamber 26 is a briquetting machine 27 wherein the ferrous sulphate monohydrate is formed into cakes for ease of handling, etc.

Disposed on the exterior of the sedimentation tank 16 and adjacent the bottom of the flared skirt 19 of the large conical baffle 18 is a hot water jacket 30. Another hot water jacket 31 is disposed peripherally of the sedimentation tank 16 at a point adjacent the discharge opening 22 in the bottom thereof. A third hot water jacket 32 is disposed between the opening 25 of the collecting chamber 26 and the float controlled valve 23 in the discharge opening 22. These hot water jackets 30-31-32 are connected successively by a line 34 which passes through a temperature controlled valve 35, the heat exchangers 14 and 5, and connects with the pickling tank 2, whereby it may be used for hot make-up water. Steam is supplied to the heat exchanger 14 and steam heater 15 by a steam line 36 which passes through a temperature controlled valve 37; and steam is supplied to the hot water jacket 30, and accordingly the hot water jackets 31 and 32, from the steam heater 15 by a pipe 38. The valve 35 controls the temperature within the tank 16 by regulating the discharge of the return pipe 34.

All of the exposed heating surfaces of the sedimentation tank 16 are covered with a suitable heat insulating medium (not shown) in order to reduce heat loss to a minimum.

The operation of the device is as follows:

From continued use, the acid in tank 2 becomes ineffective and is drained off through pipe 4 to the settling tank 8 where foreign substances in the form of sludge settle out and accumulate in the bottom of the tank. During passage through the heat exchanger 5, the temperature of the acid is lowered, this hastening the settling operation. The clear solution is withdrawn from the tank 8 by the pump 10 and passes through the pipe 13, the heat exchanger 14 and the heater 15. During its passage through the heat exchanger 14 and heater 15 the temperature of the waste pickle liquor is raised to at least 290° F. and is discharged into the pressure vessel 16 at this temperature and at a pressure of preferably 160 pounds, and at any rate—at a minimum of 120 to 140 pounds per square inch to prevent boiling of the liquor. As the liquor passes through the heater 15 and is raised to a temperature of 290° F. there is an initial tendency for the crystals to form but this tendency is discouraged by the velocity of the liquor within the pipe 13. The heated liquor enters the top of the cone 18 in the form of horizontal jets 41 which radiate from

the pipe 13 and is deflected downwardly toward the skirt 19 when it strikes the side of the cone 18. As the liquor is discharged into the space 50 its velocity is decreased and the small crystals drop downwardly out of the path of the moving liquor. As explained above, the skirt has formed in conjunction with the body of the vessel 16 a passage 20 in which an upward flow of liquor toward the return pipe 40 is created by the internal pressure of the vessel. Upon reaching the end of the skirt, the descending liquor executes a reversal of flow of 180° because of the current existing in the upwardly moving liquor in the passage 20. At the time of reversal of flow the crystals formed by chemical reaction become detached from the liquor stream and settle toward the bottom of the vessel in funnel 21 where they form into a mound-shaped mass 43. The height of this mound is maintained at a predetermined level by the float 45, which is heavier than the solution and rests on the mound 43. As the height of the mound varies, the float moves the electrical contact 46 to vary the control 47 for the valve operating motor 49 which controls the movement of the valve 23 to regulate the discharge of the formed crystals. Regulation of the height of the mound maintains the required space 50 between the mound and the skirt for the formation of crystals. As mentioned above, the initial tendency for crystal formation is imparted to the liquor in heater 15 and this tendency is increased within the inverted cone 18 to a degree where the crystals actually form and start settling out. During passage of the crystals through the liquor while settling out (which is a form of migration) crystal growth is accelerated by close association of the formative ingredients present and the resultantly formed crystals are deposited on the mound 43. As the mound increases in height, the weight of the crystals compresses the lower portion of the mass to such an extent that a large portion of the liquid remaining in the crystals is expelled and flows upwardly along the sides of the vessel to intermingle with the returning liquor in the passage 20.

The relatively dry crystals in the bottom of the funnel 21 and exit passage 22 are maintained at 290° F. by the manifold 31 of the heating system 50 as is also the expanding nozzle 25 in the crystal box 26 by the manifold 32.

The free sulphuric acid remaining after the crystals separate by sedimentation returns through the pipe 40 and the heat exchangers 14 and 5 to the pickling tank 2. A regulator 51 is included in the line 40 so that the pressure in the vessel 16 is maintained at 160 pounds which is sufficient to prevent boiling of the liquor. It will be understood that the temperature in the vessel 16 is constantly maintained at a minimum of 290° F. by means of the heating manifolds 30 and 31 and that boiling of the contents is prevented by the internal pressure which is maintained at 160 pounds by means of the pump 10 and pressure regulator 51. This maintains the liquid within the vessel in a relatively quiescent or nonturbulent condition without local disturbances, whereby the settling out of embryo crystals and their subsequent growth is not materially affected.

The monohydrate crystals discharged into the chamber 26 are formed into cakes by means of the briquetting machine 27. Fumes from the box 26 are vented through the stack 53.

If desired, a series of settling tanks could be employed to better insure continuous operation.

The efficiency of the system is increased by using the exhaust steam from the heating system of the pressure vessel 16 in the heat exchangers 14 and 5 and then discharging the steam in the form of hot condensate to the pickling tank 2. The returning liquor in the pipe 40 is heated in the heat exchangers 14 and 5.

From the foregoing, it will be perceived that the system is continuous and allows an uninterrupted return of pickle liquor freed of the ferrous sulphate monohydrate but containing free acid to the pickling tank 2; and there is permitted the maintenance of the pickle Baumé at the point most effective for the fastest and best pickling. If desired, copper sulphate may be removed from the pickle liquor returning through the pipe 40, for example, by electrolytic copper refining, but as such this forms no part of the present invention and is neither shown nor described.

While I have shown and described a specific embodiment of the present invention, it will be seen that I do not wish to be limited exactly thereto, since various modifications may be made without departing from the scope of the invention as defined in the appended claims.

I claim:

1. The continuous method of producing ferrous sulphate monohydrate from pickle liquor containing acid, which includes heating the pickle liquor to above approximately 290° F., while maintaining the liquor at a pressure sufficient to prevent formation of steam, directing flow of the heated pickle liquor into an enlarged pressure vessel so as to reduce the velocity of the pickle liquor and reversing the flow in said pressure vessel so as to cause the crystals formed at said temperature to separate by sedimentation, separating out the ferrous sulphate monohydrate thus formed while maintaining the liquor at the above temperature and pressure, and withdrawing residual liquor and free acid from the pressure vessel.

2. The continuous method of producing ferrous sulphate monohydrate from pickle liquor containing acid, which includes heating the pickle liquor to above approximately 290° F. while main-

5 taining the liquor at a pressure sufficient to prevent formation of steam, directing flow of the heated pickle liquor into an enlarged pressure vessel so as to reduce the velocity of the pickle liquor and reversing the flow in said pressure vessel so as to cause the crystals formed at said temperature to separate by sedimentation, separating out the ferrous sulphate monohydrate thus formed while maintaining the liquor at the above temperature and pressure, and withdrawing residual liquor and free acid from the pressure vessel.

10 3. The continuous method of producing ferrous sulphate monohydrate from pickle liquor which includes heating the pickle liquor to above approximately 290° F. while maintaining the liquor at a pressure sufficient to prevent formation of steam, directing flow of the heated pickle liquor into an enlarged pressure vessel so as to reduce the velocity of the pickle liquor and reversing the flow in said pressure vessel so as to cause the crystals formed at said temperature to separate by sedimentation, separating out the ferrous sulphate monohydrate thus formed while maintaining the liquor at the above temperature and pressure, and withdrawing residual liquor from the pressure vessel.

15 4. The continuous method of producing ferrous sulphate monohydrate from pickle liquor which includes heating the pickle liquor to above approximately 290° F. while maintaining the liquor at a pressure sufficient to prevent formation of steam, directing flow of the heated pickle liquor into an enlarged pressure vessel so as to reduce the velocity of the pickle liquor and reversing the flow in said pressure vessel so as to cause the crystals formed at said temperature to separate by sedimentation, separating out the ferrous sulphate monohydrate thus formed while maintaining the liquor at the above temperature and pressure, and withdrawing residual liquor from the pressure vessel.

20 45 DEXTER EDGE.